

# United States Patent Office

2,702,738

Patented Feb. 22, 1955

1

2,702,738

## PROCESS OF PREPARING FERROUS CHLORIDE FROM MIXED CHLORIDES OF IRON AND NICKEL

Marion Ernest Graham, Parma, and Edward A. Beidler, Columbus, Ohio, assignors, by mesne assignments, to Republic Steel Corporation, Cleveland, Ohio, a corporation of New Jersey

No Drawing. Application June 17, 1952,  
Serial No. 294,058

1 Claim. (Cl. 23—87)

The present invention relates to liquid phase separation of  $\text{FeCl}_2$  and  $\text{NiCl}_2$  to produce metallic nickel and substantially pure ferrous chloride.

As such, the present invention is related to our co-pending applications, Serial Nos. 160,821 and 160,822, both filed May 8, 1950, now U. S. Patent 2,677,593 and U. S. Patent 2,677,606 respectively, each issued May 4, 1954 and relating respectively to separation of ferrous chloride from material containing ferrous chloride and nickel chloride in the solid and/or liquid phase, and separation of ferrous chloride from material consisting essentially of ferrous chloride and metallic nickel. The present invention distinguishes from these two co-pending applications, in that application Serial No. 160,821 is limited to removal of the ferrous chloride from the reaction zone by vaporization of the ferrous chloride, the metallic nickel remaining behind and being separately removed. The present application is now limited to the remaining metallic constituents being physically separated from the reaction zone to leave therein a bath of substantially pure  $\text{FeCl}_2$ .

The present application distinguishes from application, Serial No. 160,822 in that the starting material in Serial No. 160,822 contains metallic nickel and substantially no nickel chloride and it is desired to prevent any conversion of the metallic nickel to nickel chloride; while in the present application the starting material contains nickel chloride, which it is a principal purpose of the process to convert to metallic nickel.

The present application is one of a group of seven co-pending applications, all the inventions of the same inventors, four of these cases relating to nickel and reactions involving nickel and the other three relating to cobalt and reactions involving cobalt. The cases may be compared and distinguished as follows:

a. Ser. No. 160,821, filed May 8, 1950, now U. S. Patent 2,677,593, issued May 4, 1954, relates to treating a starting material in the non-gaseous (liquid and/or solid) form and consisting essentially of  $\text{NiCl}_2$  and  $\text{FeCl}_2$ , and wherein there is more  $\text{FeCl}_2$  than  $\text{NiCl}_2$ . This starting material is treated in a reaction or sublimation zone, in the presence of a certain amount of metallic iron, to produce a final product which is vaporized  $\text{FeCl}_2$ , removed from the sublimation zone as such, leaving only metallic iron and metallic nickel in the sublimation zone.

b. Ser. No. 210,433, filed February 10, 1951, now U. S. Patent 2,677,594, issued May 4, 1954, relates to treating a starting material, essentially the same as Ser. No. 160,821, except that in this instance the starting material is introduced into the reaction zone in a solely gaseous state. The reaction and the final products are substantially the same as in Ser. No. 160,821.

c. Ser. No. 160,822, filed May 8, 1950, now U. S. Patent 2,677,606, issued May 4, 1954, relates to the preventing or minimizing of a possible back reaction. The starting material consists essentially of ferrous chloride and metallic nickel. It is desired to separate these materials without permitting, or at least minimizing, a possible back reaction therebetween which would produce nickel chloride and metallic iron. To do this, the starting material is introduced into a reaction or sublimation zone in which metallic iron is present. The starting material as introduced into this zone is in a non-gaseous state. The final products are substantially pure ferrous chloride vapor, which is removed from the zone

2

as such, and metallic nickel and metallic iron which remain in the zone.

d. Ser. No. 294,058, filed June 17, 1952 (the present application) discloses a process for treating a starting material substantially the same as in Ser. No. 160,821. This case has been amended so as to preclude the claims reading upon separation of the products of the reaction by vaporization as in Ser. No. 160,821; but in this case the separation following the reaction is effected by withdrawing the metallic nickel produced (by a reaction the same as in Ser. No. 160,821) by withdrawing massive pieces of iron, to which the deposited nickel adheres physically, from the fused bath of the starting materials. Neither the ferrous chloride nor any nickel chloride present is intentionally volatilized. This application is junior to application Ser. No. 160,821, so that the only subject matter claimable therein is subject matter which cannot be supported by the disclosure of Ser. No. 160,821; all the common subject matter being claimed in Ser. No. 160,821.

e. Ser. No. 291,816, filed June 4, 1952, now U. S. Patent 2,677,595, issued May 4, 1954, is the first of the three cobalt applications and is the cobalt counterpart of the nickel case, Ser. No. 160,821, distinguishing therefrom by being directed to cobalt and its chloride, rather than nickel and its respective chloride. This case is further distinguished in the degree of purity of the sublimate.

f. Ser. No. 320,835, filed November 15, 1952, now U. S. Patent 2,677,596, issued May 4, 1954, is the cobalt counterpart of nickel case, Ser. No. 210,433. It distinguishes from cobalt case Ser. No. 291,816 in the same way discussed above as to the respectively corresponding nickel cases, while distinguishing from its corresponding nickel case, Ser. No. 210,433, by the differences between cobalt and nickel.

g. Ser. No. 321,514, filed November 19, 1952, now U. S. Patent 2,677,597, issued May 4, 1954, is the cobalt case corresponding to the nickel case Ser. No. 160,822. It distinguishes from the other cobalt cases as discussed above in respect to the respectively corresponding nickel cases, while distinguishing from its nickel counterpart, Ser. No. 160,822, by the differences between nickel and cobalt.

Summarizing the present invention for the purposes of setting forth the novelty therein in respect to the closest known prior art, the present invention comprises treating a fused salt mixture, consisting essentially of  $\text{FeCl}_2$  and  $\text{NiCl}_2$ , and wherein there is at least about 50%  $\text{FeCl}_2$  by bringing into contact with a molten bath of these two salts some metallic iron, the amount to be at least enough to combine chemically with all the chlorine initially present in the fused salt bath in the form of  $\text{NiCl}_2$ ; in other words, the stoichiometric proportion or ratio of metallic iron as compared with  $\text{NiCl}_2$  for reaction in accordance with the equation:



Preferably, however, in order that the exchange reaction set forth in the equation above be carried on to substantial completion and in a relatively short time, for example, usually about 10 to 15 minutes, there should be at least 1.5 times the stoichiometric quantity of iron required as aforesaid. The temperature at which the molten bath and the iron is maintained should be such that the materials of the molten bath will remain in the liquid state, i. e., from about 1300° F. to about 1800° F.

Following the substantial completion of the reaction aforesaid, the ferrous chloride initially present, plus that formed by the reaction aforesaid, may be separated from the remaining solid metallic material by any physical separation.

The closest known prior art to the subject matter of the present invention is the three patents to Kroll, Nos. 2,396,792-3-4, all granted March 19, 1946. In all these patents the stated purpose was to purify metallic nickel by taking a body of metallic nickel, comminuting it if necessary, so as to convert the body into finely divided powder form, and then treat the powdered nickel thus prepared so as to eliminate therefrom metallic impurities, one of which was stated to be iron. The impurities in most cases were present in a total amount of not over

3%, this representing the total of all metallic impurities and not merely iron. One exception to this was in Patent No. 2,396,792, in an example given in the first column on page 3, wherein the nickel powder contained 15% iron.

In all cases the reaction relied upon for the elimination of the metallic iron was  $Fe + NiCl_2 \rightleftharpoons Ni + FeCl_2$ . From the way this equation was given and from the accompanying description in the patent, this was acknowledged to be a reversible reaction.

In Patent No. 2,396,792 the powdered impure nickel was placed in suspension in a bath of fused potassium chloride and sodium chloride in the proportion of 60/40 KCl/NaCl. The molten bath was made up in one example, at least, with the KCl/NaCl mixture about three times the weight of the metal introduced therewith. Further, in accordance with this patent, nickel chloride ( $NiCl_2$ ) was added to the molten bath, so that the resulting fused bath thus produced would be 25% to 50% nickel chloride by weight. The temperatures stated were about 500° C. to about 1000° C. In the most extreme case, that is wherein iron was present to the extent of about 15% of the metal aforesaid, the patentee stated that in about one hour 90 to 95% of the iron would be converted to ferrous chloride by the reaction above given.

In Kroll Patent No. 2,396,793, the bath was made up substantially as given above except that no nickel chloride as such was deliberately added. In accordance with the process disclosed in this patent, however, gaseous chlorine was bubbled through the bath for reaction with the constituents thereof. This was stated to chloridize some of the nickel, and either directly or indirectly to chloridize the iron present. The direct chloridizing of iron would result in ferric chloride. The indirect chloridizing of the iron was effected by first chloridizing metallic nickel to form  $NiCl_2$ , and then permitting the  $NiCl_2$  thus formed to react with metallic iron in suspension in the bath in accordance with the same equation as given above to reform metallic nickel and to convert the iron to  $FeCl_2$ . It was further taught that if additional steps of bubbling chlorine through the bath were carried on,  $FeCl_2$  in the bath would be chloridized to  $FeCl_3$ , which in turn could act in a secondary manner to chloridize some of the metallic iron in the bath and be itself reduced to  $FeCl_2$ .

The present process distinguishes from these disclosures, first in that the purpose is to obtain substantially pure  $FeCl_2$ . As distinguished from this, Kroll either puts in or obtains by his chloridizing action more  $NiCl_2$  than is disposed of by the reaction aforesaid, so as to eliminate as much of the iron as he can, while leaving an excess of  $NiCl_2$  in the bath. The present purpose is to eliminate a major part and preferably substantially all the  $NiCl_2$ , so that all the remaining water-soluble constituents will be substantially pure ferrous chloride, and preferably to have in contact with the fused bath a substantial amount of excess iron, which may be removed as such at the completion of the operation in a manner which will be hereinafter described.

As a second major difference between the process of Kroll and the present process, Kroll in the instances of both these patents uses a fused salt bath including large proportions of such salts as KCl and NaCl. In the present process the fused salt bath contains substantially no KCl or NaCl (except possibly as trace impurities), and consists essentially of  $NiCl_2 + FeCl_2$ .

As a third major difference in the process itself apart from its purpose, the present process starts with at least about 50%  $FeCl_2$ , while the concentration of this material in any bath contemplated by Kroll, either before, during, or after the reaction, in accordance with his teachings, would never contain any concentration of ferrous chloride even approaching 50%.

This last difference points up an unexpected action which takes place in accordance with the present process. Since the  $FeCl_2$  is never removed from the bath during the continuance of the reaction, the fact that this equation is a reversible one would indicate that the reaction, particularly, as shown by Kroll, in the presence of substantial amounts of  $FeCl_2$ , would never approach completion from left to right as given above. Furthermore, the ratio of  $Fe_2Cl_2$  to  $NiCl_2$ , as the reaction proceeds towards completion, approaches infinity. These two factors, taken in conjunction with the above accepted principles, would indicate that no result approaching a complete conversion of  $NiCl_2$  to metallic nickel and  $FeCl_2$  would be

possible. Notwithstanding this reasoning, it has been found, under the conditions present in accordance with the present process, that substantially complete conversion is in fact effected, so that in a period of about 10 to 15 minutes (as contrasted with Kroll's one hour period for relatively incomplete conversion) the concentration of nickel chloride in the fused bath is reduced to such a small amount as to be substantially zero, within the limits of accuracy of the analytical determinations which have been made therefor. In other words, this concentration in the remaining non-metallic material is such that the amount of nickel (calculated as metal) therein is less than 0.03%.

Turning now to the details of the present process, the starting material in accordance therewith comprises a molten bath consisting essentially of  $NiCl_2$  and  $FeCl_2$  and wherein there is at least about 50% by weight  $FeCl_2$ . This salt bath may be prepared in any desired manner from any mixtures of these two salts obtained from any source. The salt bath contains nothing else but these two salts, with the possible exception of relatively small or trace amounts of other materials.

In this bath there is provided an amount of iron for reaction therewith. It may be that this iron, which must be in metallic form, may in some way be initially present with the constituents of the bath prior to the fusion thereof. On the other hand, the iron may be introduced into the bath subsequent to the fusion of the other constituents thereof. The iron may be in any one or more of the following forms: (a) as one or more solid massive bodies, for example, one or more iron rods extending into the bath, (b) as a solid material providing a relatively large surface per unit of weight, such, for example, as a body of steel wool or a body of sponge iron, or (c) iron in relatively finely divided powdered form, irrespective of the manner of preparation or source of that powder. Any mixtures of the several forms of iron may be used if desired.

As to the amount of iron which must be present, in accordance with the present invention, there is required at least the stoichiometric equivalent amount of iron required for chemical reaction in accordance with the equation given above with all the chlorine initially present in the bath in the form of nickel chloride. From the point of view of the preferred practice of the process, however, the amount of iron is preferably substantially greater than the mere equivalent or stoichiometric amount and is at least about 1.5 times this stoichiometric or equivalent amount. On the other hand, there is no definite upper limit for the amount of iron which may be present. Thus, if an amount of iron were present, for example, in the form of one or more large masses, many times the amount necessary for conversion as aforesaid, the process is fully operative. The practical limit, therefore, is dependent upon the convenience of operation and the size of the equipment in which the process is to be carried on. Conceivably, also the process could be carried on in an iron tank or container of some kind, so that the iron would be provided by the container in which the process is carried on. This, however, is not usually desired as the process consumes some of the iron, so that the container would have a relatively short life in repeatedly carrying on the process.

The temperature for the reaction is any temperature within the general range of about 1300° F. to about 1800° F. These temperature limits are chosen as follows. The low limit of about 1300° F. is a point about or just above the melting point of the salts making up the bath aforesaid. Thus, at least this temperature is required in order that the bath be kept in a molten state, which is, of course, one of the essential factors of the present invention. The high limit again is dictated by the requirement that the bath be kept molten, this high temperature limit being about or slightly below the boiling point of mixtures of ferrous chloride and nickel chloride at atmospheric pressure. It is noted in this connection that the boiling point of a mixture of ferrous chloride and nickel chloride is above the boiling points of each of these materials alone. On the other hand, if for some reason it were desired that the high temperature limit be higher or lower, this could be effected by some control of the absolute pressure effective on the molten bath during the operation, which will in turn control the boiling point thereof in a way which will be obvious to those skilled in the art. Thus, if

it were desired to conduct the operation at some higher temperature, for example, 2000° F., sufficient super-atmospheric pressure could be employed within a closed reaction chamber or zone to keep the components of the molten bath liquid even at such a relatively high temperature. In general, the temperatures are such that the constituents of the bath remain in liquid form and do not volatilize to any substantial extent.

Due to the fact that ferrous chloride and nickel chloride are both subject to oxidation at relatively high temperatures, it is practically necessary that a non-oxidizing atmosphere be maintained above the molten bath during the present process. Such an atmosphere may conveniently be nitrogen.

The time necessary for conversion of the nickel chloride to metallic nickel and ferrous chloride in accordance with the present invention, has been found to be quite short, in the order of magnitude of 10 to 15 minutes in most cases, as will appear in greater detail from the following examples.

No particular theory of operation of the present process tending to explain how the apparently anomalous results are in fact obtained, as compared with what would be expected from the teachings of the Kroll patents and from mass action principles, can be given herein as these explanations are not known at this time. It can only be supposed, however, that the unexpected results must be due in a large measure at least to the actual differences between the present process and the processes specifically disclosed by Kroll and outlined above. In this connection, it is noted that Kroll Patent No. 2,396,794 does not relate to liquid phase operations at all, but rather is restricted to solely solid phase reactions.

Following the substantial completion of the reaction aforesaid, the ferrous chloride originally present, plus that formed by the reaction, is separated from the remaining solid metallic materials. If the iron is introduced as one or more massive bodies, such as rods, the remaining portions of these rods, to which the deposited nickel will adhere, may be lifted bodily from the bath. In the event that the iron is introduced into the molten bath in the form of a body of steel wool or of sponge iron, the remainder of such body respectively with deposited nickel adhering thereto may be lifted out of the molten bath. These expedients may be termed physical separation.

The practice of the present invention and the practical limits thereof are further illustrated by the following examples:

#### Example I

This example illustrates the effect of providing in contact with the molten mixture of  $FeCl_2$  and  $NiCl_2$ , an amount of metallic iron equivalent to at least 50% more than the amount of iron that would be theoretically necessary to react with all the chlorine present in the molten mixture in the form of  $NiCl_2$ . A charge, consisting of molten  $FeCl_2$  and  $NiCl_2$  in the ratio of 30 parts by weight of  $FeCl_2$  to one part by weight of  $NiCl_2$ , was maintained at a temperature of 1500° F. in a protective atmosphere of nitrogen. Sufficient iron in the form of steel wool was immersed in this molten bath to provide in contact with the molten material, 1.5 times the amount of iron theoretically necessary to react with all the chlorine present as  $NiCl_2$ . At the end of 15 minutes, the steel wool was removed from the molten bath and was found to have exhausted the nickel content thereof as the bath was found to be substantially free of  $NiCl_2$ . The bath, when analyzed, had a nickel content of less than 0.03% which was the limit of error of the analytical method used.

The effect of providing sufficient metallic iron in contact with the molten material upon the degree of completion of the desired reaction is seen by comparing the above result with the results obtained by providing in contact with a molten bath, having the same initial composition of  $FeCl_2$  and  $NiCl_2$ , and at the same temperature, only sufficient metallic iron to equal the amount theoretically required to react with the chlorine present as  $NiCl_2$ . It was found in this case that, even after 120 minutes of contact between the metallic iron and the molten mixture, this mixture, which originally contained 3.3%  $NiCl_2$ , still contained about 0.29%  $NiCl_2$ .

Thus, if the required purity of the  $FeCl_2$  product of the process permits of 0.29%  $NiCl_2$ , then the stoichiomet-

ric amount of iron may be used; while if a higher purity  $FeCl_2$  is required, a greater proportionate amount of metallic iron should be used as aforesaid.

#### Example II

The desired exchange reaction between metallic iron and molten  $NiCl_2$  may be brought to substantial completion, in a relatively short time, by the method of the present invention, at any temperature within the range in which the mixture of  $FeCl_2$ - $NiCl_2$  being treated is in the molten state. When a molten mixture of  $FeCl_2$  and  $NiCl_2$ , containing 30 parts by weight of  $FeCl_2$  to one part by weight of  $NiCl_2$ , was maintained at a temperature of 1300° F. (which is just above the melting point of such a mixture of chlorides), and sufficient metallic iron in the form of steel wool to equal 4 times the stoichiometric amount of iron theoretically necessary as aforesaid was maintained in contact with this chloride mixture, it was found that the molten material was substantially exhausted of its nickel content (as measured by the same test referred to in Example I) in 15 minutes.

Another mixture of these chlorides in the same proportion was treated in the identical manner at a temperature of 1800° F. It was found that the nickel content was substantially exhausted as aforesaid after 10 minutes of reaction time.

#### Example III

The metallic iron used to react with the nickel chloride may be provided in any convenient form, such as steel wool, which was used in the two examples given above. However, substantially identical results are obtained when the iron is provided in other forms. For example, it was found that when sufficient finely divided iron powder to make up 4 times the stoichiometric amount of iron theoretically necessary to react with all the chlorine present in the molten mixture in the form of  $NiCl_2$  was added to a molten mixture of  $FeCl_2$  and  $NiCl_2$ , containing these chlorides in the proportion of 30 parts by weight of  $FeCl_2$  to one part by weight of  $NiCl_2$ , at a temperature of 1500° F., substantially all of the nickel content of the molten bath was exhausted as aforesaid in 15 minutes. When the same amount of metallic iron in the form of a solid iron rod was immersed in a chloride mixture of the same composition at 1800° F. for 10 minutes, it was found again that the nickel content of the molten bath had been exhausted as aforesaid; but that this time the metallic nickel had deposited in the form of a coating on the iron rod. It was found that the deposit on the surface of the iron rod appeared to be, at least in part, an iron-nickel alloy.

#### Example IV

Although the invention finds most of its application in the treatment of the  $FeCl_2$ - $NiCl_2$  mixtures, which are relatively poor in  $NiCl_2$ , it is equally applicable to compositions containing as much as 50%  $NiCl_2$  by weight. In this case somewhat more time is required substantially to exhaust the nickel content of such a rich bath. Thus, when a molten mixture of  $FeCl_2$  and  $NiCl_2$ , containing these chlorides in equal parts by weight, was contacted with an iron rod equivalent to four times the amount of iron theoretically necessary to react with all the  $NiCl_2$  of the mixture at a temperature of 1800° F., it was found that after 15 minutes the chloride bath still contained about 2.1%  $NiCl_2$ . However, when the reaction was carried on for 30 minutes, it was found that the nickel content of said bath was completely exhausted as aforesaid.

While we have described our process in general, and have set forth in some detail the chemical and physical requirements thereof, it is recognized that the process may be operated by the substitution of such equivalents as will suggest themselves to those skilled in the art from the foregoing disclosure. We do not wish to be limited, therefore, except by the scope of the appended claims, which are to be construed validly as broadly as the state of the art permits.

What is claimed is:

The process of separating ferrous chloride, substantially free of  $NiCl_2$ , from a starting material containing both  $NiCl_2$  and  $FeCl_2$ , and in which there is a greater amount of  $FeCl_2$  and  $NiCl_2$ , which comprises introducing said material into a reaction zone in a non-gaseous state, providing sufficient metallic iron in solid massive form

in said zone and in contact with the non-gaseous material therein to assure that there is present at least sufficient metallic iron to react with all the chlorine which is present in said zone in the form of  $\text{NiCl}_2$  to form  $\text{FeCl}_2$ , maintaining the material in said zone within the temperature range of about  $600^\circ \text{C}$ . up to but below the boiling point of  $\text{FeCl}_2$  at the pressure existing in said zone and for a time and under conditions such as to permit the completion of the reaction between all the  $\text{NiCl}_2$  present with the metallic iron to form metallic nickel and  $\text{FeCl}_2$ , the metallic nickel depositing upon the solid massive iron, and separating the metallic nickel

and iron from the ferrous chloride by physically bodily removing the solid massive iron with the metallic nickel adhering thereto to leave the separated ferrous chloride, and thereby recovering said ferrous chloride in a pure state.

## References Cited in the file of this patent

## UNITED STATES PATENTS

|           |       |               |
|-----------|-------|---------------|
| 2,396,792 | Kroll | Mar. 19, 1946 |
| 2,396,793 | Kroll | Mar. 19, 1946 |
| 2,396,794 | Kroll | Mar. 19, 1946 |